

Dec. 27, 1932.

N. GONZÁLEZ

1,892,508

LEAD PENCIL AND METHOD OF MAKING THE SAME

Filed March 27, 1931

Fig. 1.



Fig. 2.



INVENTOR  
*Narciso Gonzalez*  
Casper, Stein & Dunham  
BY  
ATTORNEYS

## UNITED STATES PATENT OFFICE

NARCISO GONZÁLEZ, OF NEW YORK, N. Y., ASSIGNOR TO EAGLE PENCIL COMPANY, OF NEW YORK, N. Y., A CORPORATION OF DELAWARE

## LEAD PENCIL AND METHOD OF MAKING THE SAME

Application filed March 27, 1931. Serial No. 525,863.

This invention relates generally to the manufacture of pencils and has reference to ways of preparing leads or crayons so as to get a good adhesion between them and an outer sheath or casing when the various parts of the pencil are glued or cemented together.

In the manufacture of pencil leads or other forms of marking material for pencils, it is customary to include in the material of which they are composed various greasy or oily materials such as tallow, stearic acid and the like. These greasy or oily materials are used in various ways and in varying proportions according to the nature or kind of mark it is desired to have the pencil make. All of them are a source of difficulty in getting a good adhesion of the marking material to the casing and, as a result, the leads often have no bond attaching them to the interior of the casing because the glue or other adhesives commonly used cannot take hold upon the greasy surfaces.

An object of this invention is to change the greasy surfaces of such leads or marking material so as to remove the greasy effect and then give the pieces of marking material a coating of a material which will prevent grease from exuding from the interior of the marking material and which coating will at the same time give a surface to which glues and cements will adhere.

My present invention considered from one aspect relates to the leads themselves as new articles of manufacture; considered from another aspect relates to the structure of the complete pencil, and from a further aspect it is concerned with a method of treating the leads.

The result indicated may be obtained in various ways but a satisfactory way of carrying out the process is stated below. That statement or description is, however, intended only to be a representative one and it is not the intention to limit the invention to any one particular way of practicing it.

The invention particularly, insofar as it relates to the complete pencil may be more fully understood by reference to the accompanying drawing wherein:

Fig. 1 is a dis-assembled view showing a pencil lead about to be assembled in its sheath, and;

Fig. 2 is an enlarged transverse sectional view through the completely assembled pencil.

After the leads have been prepared in the form they are to have when assembled in pencils they are immersed in sulphuric acid for varying periods of time depending upon the depths to which the treatment is desired to go and the concentration of the acid. Sulphuric acid has the advantage of carbonizing any organic grease and thereby removing or destroying the greasy effect. After this treatment in the acid the leads may be washed in water. This washing may be carried out in a centrifugal machine or by any other practical means. The leads are then given a second treatment with dilute sulphuric acid and while the acid is adhering to them the leads are immersed in a solution of soluble salts which by reaction with the acid will precipitate on the leads in an insoluble form. A satisfactory salt solution is one of calcium chloride but there are other materials which will answer the purpose equally as well. The insoluble precipitation of calcium sulphate on the lead will serve as a casing or seal which will prevent the greasy material in the body of the lead from exuding and will also form a very satisfactory surface for the adhesion of glue or cement when the pencil is being assembled.

The two treatments with the sulphuric acid are preferred because of the fact that a speedier operation is possible. However, the two steps may be combined, particularly if the first acid bath is sufficiently diluted, and the leads transferred directly from the first acid bath to the salt solution.

In the drawing I have used the reference numeral 10 to designate one of my completely treated leads and the numerals 11-11 to indicate the two conventional half sections of wooden sheath which are glued together about the lead. In Fig. 2, I have shown on an exaggerated scale the thickness of the coating which has been formed on the lead and the thickness of the glue which is interposed be-

tween such coating and the pencil sheath and which intimately bonds the lead coating to the sheath. Here it will be observed that the lead 10 is provided with the grease impervious coating 12 formed by the process explained above and having an outer surface which will firmly adhere to the glue indicated at 13 which unites the coating to the sheath. This glue, of course, also serves to secure the 10 two sections of the sheath together, although I have not exaggerated the space between the sheath sections to indicate this.

Results which are on the whole satisfactory have been obtained by mechanically treating 15 the surfaces of the leads to remove the surface grease and then carrying out the acid and precipitating treatment as before. However, the acid treatment is more convenient and satisfactory in results and is naturally 20 preferred.

As above stated, the invention can be carried out in various ways and it is, therefore, not desired to be limited to any particular way except as such limitations may appear in 25 the claims which follow.

What is claimed is:

1. A method of coating pencil leads which comprises treating the surfaces of the leads with sulphuric acid and then, while acid is 30 adhering to said surfaces, immersing the leads in a solution of calcium chloride.

2. A method of coating pencil leads which comprises treating the surfaces of the leads with sulphuric acid, washing the leads with 35 water, immersing the leads in a weak solution of sulphuric acid, and then immersing the leads in a solution of calcium chloride.

3. A method of coating pencil leads which comprises subjecting the leads to an acid 40 treatment, and then chemically precipitating on said surfaces an insoluble material which will resist penetration by grease.

4. A method of coating pencil leads which comprises treating the surfaces of leads containing greasy material with an acid, and then precipitating on said surfaces a reaction 45 material developed from the acid and a salt which will prevent grease from exuding from the leads.

5. A method of treating pencil leads which comprises treating the leads with an acid capable of destroying surface grease, and then coating the leads with a material which 55 will adhere to the surfaces of the lead and prevent grease from exuding through the coating.

6. A method of treating pencil leads which comprises treating the leads to remove surface grease, and then coating the leads with a material which will prevent grease from 60 exuding through the coating and which will serve as a binder between the lead and the casing when the pencil is assembled.

7. A method of treating pencil leads which 65 comprises destroying or removing surface

grease from the leads, and then chemically precipitating on the leads a coating which is impervious to grease and to which adhesives will adhere.

8. A pencil including a sheath and a lead 70 enclosed therein, said lead being inherently internally greasy throughout the length thereof and a grease impervious coating at the outer surface of the lead intimately adhesively bonded to the sheath. 75

9. A lead pencil including a lead, a sectional sheath thereabout and a binder means interposed between them preventing exudation of grease from the lead and intimately 80 adhesively attached to the sheath.

10. A lead pencil including a sheath, a core 85 of marking material of the type normally subject to grease exudation, adhesive between the core and sheath, and means preventing grease exudation from the core and establishing an intimate bond between the core and the adhesive material.

11. As a new article of manufacture a pencil lead having a grease impervious coating. 90

12. As a new article of manufacture a pencil lead having a grease impervious coating, the exterior surface of said coating being inherently adapted for intimate adhesive bonding to an enclosing sheath. 95

13. As a new article of manufacture a pencil lead having a coating of calcium sulphate. 100

In testimony whereof I hereto affix my signature.

NARCISO GONZÁLEZ.

100

105

110

115

120

125

130